# EUROPEAN PATENT SPECIFICATION

(11) **EP 0 819 053 B1**
(45) Date of publication and mention of the grant of the patent: **02.06.1999**
(21) Application number: 96907796.5
(22) Date of filing: 09.04.1996
(51) Int. Cl.: B31D 3/02

(54) **A METHOD FOR MAKING EXPANDED PAPER HONEYCOMB CORE MATERIAL MOISTURE- OR WATERPROOF, AND THE THUS OBTAINED HONEYCOMB CORE MATERIAL**
VERFAHREN ZUR HERSTELLUNG EINES AUS PAPIER EXPANDIERTEN, FEUCHTIGKEITSBESTÄNDIGEN ODER WASSERBESTÄNDIGEN, WABENKERNMATERIALS, UND DAS SO HERGESTELLTE WABENKERNMATERIAL
PROCEDE DE FABRICATION D'UN MATERIAU EN NID D'ABEILLES EN PAPIER EXPANSE, IMPERMEABLE A L'HUMIDITE OU A L'EAU AINSI QUE LE MATERIAU EN NID D'ABEILLES OBTENU

(30) Priority: 07.04.1995 NL 1000088
(43) Date of publication of application: 21.01.1998
(73) Proprietor: BESIN B.V., 3851 BD Ermelo (NL)
(72) Inventor: DIDERICH, Philippus, Ludovicus, Maria, NL-3851 BD Ermelo (NL)
(74) Representative: Ferguson, Alexander
(86) International application number: NL9600150
(87) International publication number: WO9631339

(56) References cited:
- FR-A- 2 171 949
- FR-A- 2 568 513
- NL-A- 6 805 968
- US-A- 2 731 379

## Description

The invention relates to a method for making expanded paper honeycomb core material moisture- or waterproof, as well as the honeycomb core material obtained by using this method.

Paper honeycomb core material is often used as a stiff and light construction material. In a number of applications it is necessary for the paper honeycomb core material to be moisture- or waterproof, as for example in construction panels for outside use, for use in transport and for use in floors and such like. In these cases, the honeycomb core material is usually delivered in moisture- and waterproof condition, after which the user himself provides one or both sides of the honeycomb core material with a cover layer of plastic or metal, for example.

Paper honeycomb core material is obtained by glueing a number of strips of paper onto each other at certain places, and, after the glue has dried, expanding this parcel of paper by pulling the outer strips of paper apart laterally, thus obtaining the hexagonal cellular structure. After the expanded shape has been stabilized, the honeycomb core material is cut into slices of the desired thickness, which are further used as honeycomb core in honeycomb panels, for example.

It is known to make the paper honeycomb core material moisture- and waterproof after expansion by impregnating the paper. Impregnation is effected by immersing the expanded honeycomb core material in a solution of formaldehyde and water. In the known processes immersion usually takes place a number of times in order to apply the desired amount of resin. After immersion, the impregnated honeycomb core material must be dried with the aid of a drying facility in order to remove the surplus of water from the honeycomb core material.

This way of making paper honeycomb core material moisture-and waterproof has a number of disadvantages. Formaldehyde is a poisonous substance that makes recycling or dumping difficult. Owing to the fact that immersion has to take place a number of times, the treatment is time-consuming and elaborate, which results in high process costs. Drying, at the end of the process, is an extra step in which the solvent with formaldehydefumes must be disposed of in a safe manner.

It is an aim of the invention to provide a method for making expanded paper honeycomb core material moisture- or waterproof which overcomes these disadvantages.

According to the invention, this aim is achieved by the measure that the honeycomb core material is provided with a coating after expansion.

This brings about, that the paper honeycomb core material is provided with a sealing layer that offers an effective protection against moisture and water. The coating can be applied in one layer, so that repeated immersions are not necessary. Nor does formaldehyde have to be used any more. By applying the coating a coating-paper-coating-sandwich is obtained, which produces a lighter and stronger construction as compared to impregnated paper. This method is cheaper than the one in which strips of paper are provided with a coating before they are glued to one another and expanded, as less coating material is needed, that is not on the glued areas, and as the usual glues may be used. In addition, expenses are saved because spoilage of honeycomb core material during production has not yet been provided with the cost price raising coating.

The coating is preferably applied as a powder of a polymer material, as, in this way, it is possible to apply a coating of essentially equal thickness across the entire length of the honeycomb cells within a short time.

In an advantageous embodiment of the method, powder is applied by providing the paper honeycomb core material and the powder with an opposed electric charge, as a result of which a predetermined amount of powder can be applied to the honeycomb core material simply and quickly, by allowing the honeycomb core material to attract the powder electrically.

In this case it is advantageous to moisten the paper honeycomb core material with water before the powder is applied, as this makes it easier to give the paper honeycomb core material a suitable electric charge.

Moistening is preferably carried out by sprinkling with water, preferably such an amount of water being used, that a degree of humidity equal to 15-30 percentage by weight of the honeycomb paper is obtained. By sprinkling, the paper easily and quickly acquires an even, suitable degree of humidity. It has been established that the stated degree of humidity achieves good results in practice.

For the polymer powder, a thermosetting polyester or epoxy is preferably used, since a strong moisture- and waterproof coating can be made from a thermosetting polyester or epoxy or a mixture of the two.

In an advantageous manner the honeycomb core material is heated after the thermosetting powder has been applied, in order to let the powder turn into a hard and thick coating and to stabilize the coated honeycomb core material in the expanded state, in which the heating is preferably carried out by means of hot air or by infrared radiation in order to obtain quick and even heating.

The invention also relates to the paper honeycomb core material that is obtained with the method described above.

## Claims

1. A method for making expanded paper honeycomb core material moisture- or waterproof, **characterized in that** the honeycomb core material is provided with a coating after the expansion.

2. A method according to claim 1, **characterized in that** the coating is applied as a powder of a polymer material.

3. A method according to claim 2, **characterized in that** the powder is applied by providing the paper honeycomb core material and the powder with an opposed electric charge.

4. A method according to claim 3, **characterized in that** the paper honeycomb core material is moistened with water before the powder is applied.

5. A method according to claim 4, **characterized in that** the moistening takes place by sprinkling with water, preferably such an amount of water being used that a degree of humidity equal to 15-30 percentage by weight of the honeycomb paper is obtained.

6. A method according to one of the claims 2 up to and including 5, **characterized in that** a thermosetting polyester or epoxy is used for the polymer powder.

7. A method according to claim 6, **characterized in that** the honeycomb core material is heated after the thermosetting powder has been applied, in order to let the powder flow out into a hard and thick coating and to stabilize the coated honeycomb core material in the expanded state.

8. A method according to claim 7, **characterized in that** the heating is carried out by means of hot air.

9. A method according to claim 7, **characterized in that** the heating is carried out by means of infrared radiation.

10. Paper honeycomb core material provided with a coating that is obtained by the method described in one of the above claims.

## Patentansprüche

1. Verfahren um ausgedehntes, Papierhonigwabekernmaterial feuchtigkeitsbeständig oder wasserfest zu machen, **dadurch gekennzeichnet**, daß das Honigwabekernmaterial nach dem Ausdehnen mit einer Beschichtung versehen wird.

2. Verfahren gemäß Anspruch 1, **dadurch gekennzeichnet**, daß die Beschichtung als ein Pulver von Polymermaterial angeordnet wird.

3. Verfahren gemäß Anspruch 2, **dadurch gekennzeichnet**, daß das Pulver angeordnet wird durch das Papierhonigwabekernmaterial und das Pulver eine entgegengesetzte elektrische Ladung zu geben.

4. Verfahren gemäß Anspruch 3, **dadurch gekennzeichnet**, daß das Papierhonigwabekernmaterial vor dem Anordnen des Pulvers mit Wasser befeuchtet wird.

5. Verfahren gemäß Anspruch 4, **dadurch gekennzeichnet**, daß das Befeuchten durch das Besprühen mit Wasser stattfindet, wobei vorzugsweise eine derartige Menge Wasser benutzt wird, daß einen Feuchtigkeitsgehalt gleich an 15 - 30 Gewichtsprozentsatz vom Honigwabepapier erzielt wird.

6. Verfahren gemäß einem der Ansprüche 2 bis einschließlich 5, **dadurch gekennzeichnet**, daß einen thermoaushärtbaren Polyester oder ein Epoxid für das Polymerpulver benutzt wird.

7. Verfahren gemäß Anspruch 6, **dadurch gekennzeichnet**, daß das Honigwabekernmaterial nach dem Anordnen des thermoaushärtbaren Pulvers erhitzt wird, um das Pulver zu einer festen und dichten Beschichtung zerfließen zu lassen und um das beschichtete Honigwabekernmaterial in ausgedehnter Lage zu stabilisieren.

8. Verfahren gemäß Anspruch 7, **dadurch gekennzeichnet**, daß das Erhitzen mit Hilfe heisser Luft ausgeführt wird.

9. Verfahren gemäß Anspruch 7, **dadurch gekennzeichnet**, daß das Erhitzen mit Infrarotstrahlung ausgeführt wird.

10. Papierhonigwabekernmaterial mit einer Beschichtung versehen, mit dem Verfahren gemäß einem der vorabgehenden Ansprüche erzielt.

## Revendications

1. Procédé pour la fabrication d'un matériau de papier en nid d'abeille expansé, imperméable à l'humidité ou à l'eau, caractérisé en ce que le papier en nid d'abeille est pourvu d'un revêtement après expansion.

2. Procédé selon la revendication 1, caractérisé en ce que le revêtement est appliqué sous la forme d'une poudre d'un matériau polymère.

3. Procédé selon la revendication 2, caractérisé en ce que la poudre est appliquée en établissant au niveau du matériau de papier en nid d'abeille et de la poudre des charges électriques opposées.

4. Procédé selon la revendication 3, caractérisé en ce que le matériau de papier en nid d'abeille est humidifié avec de l'eau avant application de la poudre.

5. Procédé selon la revendication 4, caractérisé en ce que l'humidification est réalisée par aspersion d'eau, de préférence en utilisant une quantité d'eau suffisante pour conduire à un degré d'humidité compris entre 15 et 30 % en poids du papier en nid d'abeille.

6. Procédé selon l'une quelconque des revendications 2 à 5, caractérisé en ce que l'on utilise un polyester ou époxy thermodurcissable en tant que poudre de polymère.

7. Procédé selon la revendication 6, caractérisé en ce que le matériau en nid d'abeille est chauffé après application de la poudre thermodurcissable de façon à ce que la poudre s'écoule en formant un revêtement épais et dur et à stabiliser le matériau en nid d'abeille revêtu, dans un état expansé.

8. Procédé selon la revendication 7, caractérisé en ce que le chauffage est réalisé au moyen d'air chaud.

9. Procédé selon la revendication 7, caractérisé en ce que le chauffage est réalisé au moyen de radiations infrarouges.

10. Matériau de papier en nid d'abeille pourvu d'un revêtement obtenu selon le procédé de l'une quelconque des revendications précédentes.
